

Patented Mar. 2, 1937

2,072,808

UNIT A 252/512 X 2027T  
 15/15  
 x 252/514 X 2038E  
 x 252/517

Rudolph S. Bley, Elizabethton, Tenn., assignor to  
 North American Rayon Corporation, New York,  
 N. Y., a corporation of Delaware

No Drawing. Application October 11, 1934,  
 Serial No. 747,895

10 Claims. (Cl. 106—40)

The present invention relates to a process of producing dull-luster cellulosic filaments having bactericidal properties.

One object of my invention is the dispersion of an organosol, containing at least two dissimilar, colloidal metals into cellulosic spinning solutions to form subsequently by extrusion into conventional setting baths or air delustered, bactericidal filaments.

10 Another object of my invention relates to a pre-irradiation of the organosols and colloidal metals with ultra-violet rays.

15 A third object of the present invention has to do with a novel product per se, namely dull-luster, bactericidal filament of cellulosic origin.

Other objects of my invention will become apparent to those skilled in the art from a study of the following specification.

I am well aware that it has, heretofore, been proposed to use colloidal metals as disinfectants (vide, "Rideal, Disinfection and Sterilization", 1921, pages 206-9), and to impregnate textile fibers with metallic salts and colloidal hydroxides (vide U. S. Patents Nos. 22,362, 1,482,416, 1,536,254 and 1,717,483) to prevent fungous growth. I am also aware that it has, heretofore, been proposed to add hydrocarbons, vegetable and mineral oils, pigments, etc. to cellulosic spinning solutions to produce dull-luster filaments, but I believe myself to be the first inventor to produce dull-luster, bactericidal products of cellulosic origin.

I have found by experimentation that colloidal metals per se have a relatively weak sterilizing effect, especially when being imbedded in cellulosic filaments. After a thorough investigation of the effect of colloidal metals as well as colloidal metal compounds upon non-pathogenic microorganisms such as bacteria and molds, I have found that the bactericidal effect of the aforementioned substances can be substantially increased and accelerated by distributing two or more dissimilar, colloidal metals into cellulosic spinning solutions.

In order to increase and/or accelerate the bactericidal properties of colloidal metals, it is necessary to select at least two dissimilar metals.

When microorganisms, such as bacteria, molds, etc., are distributed in a liquid phase and subsequently a solid phase, such as colloidal metal, is added thereto, they are killed after a while and the liquid becomes sterile. The time consumed to paralyze the protoplasm of microorganisms naturally depends upon the species of microorganisms treated, the chemical composition and temperature of the nutritive solution and the amounts and chemical properties of the colloidal metals used as disinfectants. The physico-chemical principles underlying this sterilization are unknown, although the theory has been advanced that the colloidal metal particles become ad-

sorbed to the membranes of the microorganisms and in turn prevent proper assimilation of nutritive substances. Other investigators have claimed that invisible rays are emitted by the colloidal particles which paralyze protoplasm. I have been unable to definitely find the cause why cells of microorganisms are much more rapidly killed in the presence of two or more dissimilar, colloidal metals.

Table 1 depicts the results obtained by using 10 various colloidal substances, in accordance with the present invention, to sterilize aqueous suspensions of *Bacillus coli*, an organism commonly appearing in fouling liquids. To obtain comparable results, aqueous suspensions of *Bacillus coli* 15 were prepared by inoculation into sterile water. Subsequently, equal amounts of this bacterial suspension were transferred by means of a platinum loop into test tubes containing identical quantities of sterile beef broth gelatine. After 20 thoroughly shaking each inoculated test tube to evenly distribute the bacterial cells in the nutritive, molten gelatine an equal amount of disinfectant was added to the test tubes and the same 25 incubated, after thorough shaking, at a temperature of about 37.5° C. To determine the exact period of time necessary to sterilize the cultures, each tube was opened at five minute intervals 30 under sterile conditions and a loop of the cultures inoculated into new sterile beef-broth gelatine 35 tubes. The first tube of each series, showing no growth on incubation for several days, was considered the characteristic one for each disinfectant tested.

Table I

*Bacillus coli* cultivated in beef broth-gelatine at 37.5° C.  
 One loop of bacterial suspension inoculated into every test tube containing 10 cc. of gelatine. 0.1 g. of disinfectant in 1 cc. of distilled water and 0.01 g. gelatine as protective colloid.

| Disinfectant                      | Times of treatment in minutes |    |    |    |    |    |    |    |
|-----------------------------------|-------------------------------|----|----|----|----|----|----|----|
|                                   | 0                             | 10 | 20 | 30 | 40 | 50 | 60 | 70 |
| Colloidal copper.....             | X                             | X  | X  | X  | -  | -  | -  | -  |
| Colloidal silver.....             | X                             | X  | X  | X  | X  | X  | -  | -  |
| Colloidal silver plus copper..... | X                             | X  | X  | -  | -  | -  | -  | -  |
| Colloidal gold.....               | X                             | X  | X  | -  | X  | -  | -  | -  |
| Colloidal gold plus copper.....   | X                             | X  | X  | -  | -  | -  | -  | -  |

X indicates that *Bacillus coli* is growing.  
 - indicates that *Bacillus coli* is dead.

When using composite disinfectants, equal amounts of each ingredient were used to make up 0.1 g. of disinfectant, for example 0.05 g. copper plus 0.05 g. silver, etc., although the ratio of the ingredients may be varied at will.

I have, furthermore, found that colloidal metals, irradiated with ultra-violet rays, prior to being used as disinfectants, have a greater bac-

tericidal power than non-irradiated ones. Although ultra-violet rays stimulate the aforementioned colloidal disinfectants to a higher degree than daylight, it is to be noted that a prolonged irradiation fails to increase the bactericidal effect of a disinfectant beyond a fixed limit. This limit varies for each metal, and combinations thereof, and it must be determined by experiment, in other words, each colloidal agent has a definite optimum time of irradiation. Over-exposure to ultra-violet rays does not deleteriously affect the colloidal disinfectants, but it should be avoided for reasons of economy. I am unable to define the complex reactions which evidently take place in such irradiated dispersions, but I have definitely found that the agents, cited above, substantially increase their bactericidal powers after being irradiated. This stimulation by means of irradiation is so pronounced that even the walls of glass flasks in which they are kept acquire bactericidal properties. When, for example, all colloidal metals are removed from such a flask by rinsing and the same is filled with a suspension of virulent bacteria, the bacteria will be killed after standing for some time. This experiment can be repeated several times, the glass walls acting as disinfectants in the absence of colloidal particles; at least I have been unable to detect with the microscope any particles adsorbed to the glass walls of such flasks. Although I am unable to explain this phenomenon, a marked increase of the bactericidal power of my agents is obtained by pre-irradiation. Table II depicts some results obtained by this method.

35

Table II

## Effect of irradiation

All dispersions were irradiated with ultra-violet rays in open glass dishes prior to being used as disinfectants. After inoculation, the tubes were kept in a dark incubator. (See Table I.)

40

| Disinfectant                                                                                 | Periods of time for complete sterilization in minutes |                |
|----------------------------------------------------------------------------------------------|-------------------------------------------------------|----------------|
|                                                                                              | Irradiated                                            | Not irradiated |
| Colloidal copper                                                                             | 20                                                    | 30             |
| Colloidal silver                                                                             | 55                                                    | 60             |
| Colloidal silver plus copper                                                                 | 18                                                    | 20             |
| Glass flask after removing all disinfectants with water, first trial                         | 120                                                   | -----          |
| Second trial after removing bacterial suspension and adding a new culture of living bacteria | About four hours                                      | -----          |

55 Similar results were obtained with spores of *Mucor* and *Oidium* species, although they are more resistant to destruction. After standing in the dark for 14 days, the irradiated colloidal disinfectants were again compared with the non-irradiated ones. The pre-irradiated disinfectants had retained greater sterilizing powers than the non-irradiated ones. It is to be noted, however, that the sterilization, obtained by pre-irradiation, slowly abates on standing, and that it may 60 be revived by a second irradiation, etc.

65 The colloidal dispersions may be prepared by wellknown processes to form suitable disinfectants. The metals and alloys may be dispersed by electrical means and held in aqueous suspension 70 by adding thereto suitable protective colloids, such as gelatine, agar, gums, alginates, casein, soluble silicates, protalic acid, etc., before being suspended in oils. Colloidal metals may also be formed by chemical precipitation in aqueous solutions. Subsequently, the by-products may be re-

75 moved by dialysis, the dispersions dried at low temperatures and suspended in oils with or without protective colloids, to form metal organosols. Two or more colloidal metals may be simultaneously precipitated in the aforementioned manner. 80 dialyzed, dried and suspended in oils. Collodial copper, for example, may be prepared in the following manner. A 20% aqueous solution of copper sulphate, containing about 10 to 20% saccharose, is boiled for a few minutes and subsequently diluted with an equal amount of distilled water, this comprising solution No. 1. Solution No. 2 consists of a 14% aqueous solution of sodium or potassium hydroxide. Solution No. 3 is prepared by adjusting sulphuric acid so that 1 cc. thereof corresponds to 2 ccs. of the hydroxide solution. Solution No. 4 is obtained by dissolving approximately 5 g. of gelatine in 100 ccs. of distilled water. After having prepared solutions 1 to 4, 10 ccs. of solution No. 1 are mixed with 40 ccs. 90 of solution No. 4 and the mixture boiled on a water bath for a few minutes. About 5 to 6 ccs. of solution No. 2 are added to the hot mixture to precipitate colloidal cuprous hydroxide. This cuprous oxide is purified by dialysis, dried and suspended 95 in suitable organic compounds to form a cuprous hydroxide organosol to which other colloidal metals may be added. To form colloidal copper from cuprous hydroxide, the solution is again boiled and subsequently 3 ccs. of solution No. 3 100 added thereto. Red colloidal copper is spontaneously precipitated. This colloidal copper may be treated, as set forth above, to produce a copper organosol. Instead of using sulphuric acid to form colloidal copper, any acid may be 105 employed in which colloidal copper is insoluble. Such colloidal metals and colloidal metal alloys may be also prepared by reducing water-soluble metal salts with aldehydes, p-aminophenol, etc. 1 g. of gold chloride for example, is dissolved in a 110 few ccs. of distilled water and added to 500 ccs. of a 10% aqueous solution of vinyl alcohol. After addition of a mixture of 40 ccs. of formaldehyde and 40 ccs. of n-sodium carbonate solution, colloidal gold is precipitated which may be purified 115 by dialysis. The purified colloids are dispersed in oils, hydrocarbons, etc., by means of ball or colloid mills.

120 Organosols of metals may also be prepared in the following manner. 10 g. of silver nitrate, for example, are mixed with about 100 g. of a sterol, such as cholesterol, phytosterol, etc., and the mixture carefully heated to about 250° C. until a silver mirror appears on the surface of the composition. The heat-reaction products of sterols containing colloidal silver may be suspended in oils, such as olive oil, Turkey red oil, mineral oils, animal oils, etc. Suitable protective colloids, such as oil-soluble soaps, naphthenates, etc., may be added to stabilize the organosols. When such metal organosols are incorporated into cellulosic spinning solutions, bactericidal filaments are obtained 125 which are simultaneously delustered.

## Example I

130 Two or more dissimilar, colloidal metals, for example, colloidal copper and zinc are dispersed in a vegetable, mineral or animal oil, to form an organosol which is emulsified with a conventional viscose spinning solution. The amounts of colloidal metals in an organosol, i. e., the solid phase of the organosol, may be varied at will. The amounts of oils, hydrocarbons, etc., to be added to the spinning solution, constituting the liquid phase of the organosol, may also be varied at will. 135

Thus, it is possible to produce more or less de-lustered, as well as more or less bactericidal filaments and/or yarns. In order to prevent an externally visible change in color of the finished products, the organosol is adjusted so that about 0.25 to 1.0 g. of solid phase is incorporated into about 1000 g. of a viscous solution. In this manner, it is possible to produce viscose products having the same bactericidal power and yet a different degree of luster. By varying the amount of solid phase in a given amount of liquid phase, it is possible to produce viscose products having an identical degree of luster and yet different bactericidal properties. According to the amounts of liquid and solid phases present in the finished products, they may even have the appearance of dull metals. Instead of using copper, zinc, silver, gold, etc., any combination of colloidal metals is suitable which is able to set up a sufficient potential difference in the presence of electrolytes, such as the minute salt residues present in finished cellulosic products. As soon as the finished product becomes exposed to moist air, etc., the potential difference, caused by the dissimilar metals, will be sufficient to prevent growth of microorganisms therein and thereon. Pre-irradiated metal dispersions may replace non-irradiated colloidal metals to increase the bactericidal properties of the finished product. Instead of using viscose solutions in combination with my disinfectants, it is possible to incorporate the same into any known type of cellulosic spinning solutions, such as cuprammonium cellulose, cellulose esters, cellulose ethers, etc. Care has to be taken, however, in selecting proper colloidal metals. Should a metal be incorporated which is decomposed by the spinning solution, the resulting gas will cause the formation of hollow filaments. Should such hollow filaments be desired, it is necessary to incorporate at least one easily decomposed metal together with other stable colloidal metals into the spinning solution prior to the extrusion thereof. It is also necessary that the colloidal metals are unaffected by the liquid phase of the organosol, and that this liquid phase is immiscible with the spinning solutions. To produce dull-luster filaments, the liquid phase should have a different index of refraction than the spinning solution with which it is to be emulsified. Thus, an almost unlimited number of organic liquids may be used as the liquid phases of my organosols, for example, vegetable oils, mineral oils, animal oils, hydrocarbons, essential oils, etc.

I wish to point out that the above example is merely illustrative, and I do not wish to be limited to the exact proportions set forth above, which are typical combinations, since certain of these ingredients may be omitted or replaced by others of similar nature, and the proportions within wide limits may be varied. In other words, while I have found that the colloidal metals above mentioned, give the desired results, I do not wish to be limited to the use of all of these substances and no others, nor the exact proportions and concentrations set forth above, as the omission of some ingredients or a slight variation of proportions will not adversely affect the final products, although it may vary somewhat the relative characteristics of such products, resulting from such variations. I wish to emphasize that the term "dissimilar" metals, employed in the appended claims, embraces a combination of two or more chemically different metals or alloys which set up a more or less large potential difference in the presence of minute amounts of electrolytes. These

colloidal metals and alloys are called the "solid phase" of the organosol, while the oils, hydrocarbons, in which they are dispersed are termed the "liquid phase" of the organosol. Thus the "organosol" consists of solid and liquid phases which must be substantially insoluble in and inert to the spinning solutions as well as the treatment-baths into which these solutions are extruded and otherwise treated. Modifications may be made in details of the method and product without departing from the spirit and scope of my invention, as defined by the appended claims.

I claim:

1. A cellulosic spinning solution for the manufacture of dull-luster, bactericidal cellulosic products comprising a cellulosic solution having an organosol emulsified therewith, said organosol including a plurality of colloidal, dissimilar metals dispersed in an organic liquid, said liquid being substantially immiscible with and inert to said cellulosic solution, and said metals being able to set up a potential difference in the presence of a minute amount of an electrolyte while being stable in said organic liquid and said cellulosic solution. 25

2. A cellulosic spinning solution for the manufacture of dull-luster, bactericidal cellulosic products comprising a cellulosic solution having an organosol emulsified therewith, said organosol including a plurality of colloidal, dissimilar metals dispersed in a liquid hydrocarbon, said hydrocarbon being substantially immiscible with and inert to said cellulosic solution, and said metals being able to set up a potential difference in the presence of a minute amount of an electrolyte while being stable in said organic liquid and said cellulosic solution. 30

3. A cellulosic spinning solution for the manufacture of dull-luster, bactericidal cellulosic products comprising a cellulosic solution having an organosol emulsified therewith, said organosol including a plurality of colloidal, dissimilar metals dispersed in an organic liquid and able to set up a potential difference in the presence of a minute amount of an electrolyte, said liquid being substantially immiscible with and inert to said cellulosic solution and said metals and said metals being pre-irradiated with ultra-violet rays. 40

4. A cellulosic spinning solution for the manufacture of dull-luster, bactericidal cellulosic products comprising a cellulosic solution having an organosol emulsified therewith, said organosol including a plurality of colloidal, dissimilar metals dispersed in a liquid hydrocarbon and able to set up a potential difference in the presence of a minute amount of an electrolyte, said hydrocarbon being substantially immiscible with and inert to said cellulosic solution and said metals and said metals being pre-irradiated with ultra-violet rays. 50

5. A cellulosic spinning solution for the manufacture of dull-luster, bactericidal cellulosic products comprising a viscose solution having an organosol emulsified therewith, said organosol including a plurality of colloidal, dissimilar metals dispersed in an organic liquid and able to set up a potential difference in the presence of an electrolyte, said liquid being substantially immiscible with and inert to said viscose solution and said metals. 65

6. A cellulosic spinning solution for the manufacture of dull-luster, bactericidal cellulosic products comprising a viscose solution having an organosol emulsified therewith, said organosol including a plurality of colloidal metals dispersed 75

in a hydrocarbon and able to set up a potential difference in the presence of a minute amount of an electrolyte, said hydrocarbon being substantially immiscible with and inert to said viscose solution and said metals.

5 7. A cellulosic spinning solution for the manufacture of dull-luster, bactericidal cellulosic products comprising a viscose solution having an organosol emulsified therewith, said organosol including a plurality of colloidal dissimilar metals dispersed in an organic liquid and able to set up a potential difference in the presence of a minute amount of an electrolyte, said liquid being substantially immiscible with and inert to said viscose solution and said metals and said metals being pre-irradiated with ultra-violet rays.

10 8. A cellulosic spinning solution for the manufacture of dull-luster, bactericidal cellulosic products comprising a viscose solution having an organosol emulsified therewith, said organosol including a plurality of colloidal, dissimilar metals dispersed in a hydrocarbon and able to set up

a potential difference in the presence of a minute amount of an electrolyte, said hydrocarbon being substantially immiscible with and inert to said viscose solution and said metals and said metals being pre-irradiated with ultra-violet rays.

5

9. A dull-luster, bactericidal cellulosic product containing an organosol comprising a plurality of colloidal, dissimilar metals dispersed in an organic liquid inert with respect to said metals, said liquid forming globules in the product, and said metals being able to set up a potential difference in the presence of a minute amount of an electrolyte.

10 10. A dull-luster, bactericidal cellulosic product containing an organosol comprising a plurality of colloidal, dissimilar metals dispersed in a hydrocarbon inert with respect to said metals, said hydrocarbon forming globules in the product, and said metals being able to set up a potential difference in the presence of a minute amount of an electrolyte.

RUDOLPH S. BLEY.